

March 5, 1974

W. E. SPICER

3,795,531

X-RAY IMAGE INTENSIFIER TUBE AND METHOD OF MAKING SAME

Original Filed Dec. 27, 1966



**FIG. 2**  
PRIOR ART



**FIG. 4**



**FIG. 5**

INVENTOR  
WILLIAM E. SPICER  
BY  
*John D. Nolan*  
(ATTORNEY)

1

**3,795,531**  
**X-RAY IMAGE INTENSIFIER TUBE AND METHOD**  
**OF MAKING SAME**

William E. Spicer, Portola Valley, Calif., assignor to  
Varian Associates, Palo Alto, Calif.  
Continuation of abandoned application Ser. No. 606,514,  
Dec. 27, 1966. This application Feb. 3, 1970, Ser. No.  
7,358

Int. Cl. H01j 31/49

U.S. Cl. 117—33.5 C

15 Claims

## ABSTRACT OF THE DISCLOSURE

The present invention relates in general to methods for making pick-up screens for X-ray image intensifier tubes and, more particularly, to an improved method wherein the X-ray fluorescent phosphor screen element is formed by evaporation of an alkali metal halide material in vacuum and condensing the evaporated material on an X-ray transparent portion of the X-ray intensifier tube, whereby a curved X-ray image pick-up screen is formed which has improved quantum efficiency and resolution. Such improved X-ray image intensifier tubes are especially useful for, but not limited in use to, X-ray systems and for intensifying gamma ray images obtained in applications of nuclear medicine.

## RELATED CASES

The present application is a continuation application of copending parent application 606,514 filed Dec. 27, 1966 and now abandoned and assigned to the same assignee as the present application.

Heretofore, X-ray image pick-up screens for X-ray image intensifier tubes have been made by settling phosphor particles out of a liquid slurry onto an X-ray transparent spherical dish, as of aluminum, forming the pick-up face of the evacuated image intensifier tube. While such techniques are suitable for ZnS pick-up screen materials they are generally unsuited for producing alkali metal halide screens which should provide improved X-ray quantum efficiencies. Moreover, the particulated screen produced by such settling methods has only about half the density of the bulk material and has poorer resolution than that obtainable from a screen having a higher density of the screen material. Also it would be desirable to use a screen material having higher stopping power and quantum conversion efficiency such as that provided by the alkali metal halide.

While it may be possible to form the pick-up screen of a thin slab of alkali metal halide, which has been deformed to produce the spherical shape, such a deformation of the slab of phosphor material may seriously degrade the conversion efficiency and, thus, resolution of the converted X-ray image because of the plastic deformation of the alkali metal halide.

In the present invention, the spherical pick-up screen is formed by evaporation of an alkali halide material, such as CsI, KI, NaI, RbI, CsBr, or LiI, in vacuum onto the inside of the spherical X-ray transparent pick-up face plate of the image intensifier tube. Such an evaporated pick-up screen has a density which is approximately equal to that of the bulk material and, therefore, will provide enhanced resolution and quantum conversion efficiency.

In one embodiment of the present invention, the alkali halide phosphor screen material is co-evaporated with its activator material either by evaporation of an activated alkali metal halide or by simultaneous evaporation of the alkali metal halide and its activator.

In another embodiment of the present invention, the alkali halide screen is evaporated and condensed in place

2

and subsequently activated by coating the screen with the activator, as by evaporation, and then diffusing the activator from the coating into the screen material.

The principal object of the present invention is the provision of methods for making improved X-ray image intensifier tubes.

One feature of the present invention is the provision of a method for making the X-ray pick-up screen of an image intensifier tube wherein an alkali metal halide screen material is evaporated in vacuum onto an X-ray transparent substrate, whereby a phosphor screen is produced which has improved resolution and quantum conversion efficiency.

Another feature of the present invention is the same as the preceding wherein the alkali halide material is co-evaporated with its activator material.

Another feature of the present invention is the same as the preceding feature wherein the alkali halide to be evaporated includes its activator.

Another feature of the present invention is the same as the first feature wherein the alkali halide material and its activator material are simultaneously evaporated from separate sources onto the substrate member.

Another feature of the present invention is the same as the first feature wherein the alkali halide screen, as deposited on the substrate, is activated by coating the surface of the screen with an activator material and then diffusing the activator into the alkali halide screen by raising the screen to an elevated temperature.

Another feature of the present invention is the same as any one or more of the preceding features wherein the alkali metal halide screen is annealed to remove minute residual plastic deformation of the material.

Other features and advantages of the present invention will become apparent upon a perusal of the following specification taken in connection with the accompanying drawings wherein:

FIG. 1 is a schematic line diagram of an X-ray image intensifier tube of the prior art,

FIG. 2 is an enlarged cross sectional view of a portion of the structure of FIG. 1 delineated by line 2—2,

FIG. 3 is a view similar to that of FIG. 2 depicting the pick-up screen construction of the present invention,

FIG. 4 is a schematic line diagram of an apparatus for evaporating alkali halide materials in vacuum, and

FIG. 5 is an alternative evaporator apparatus to that depicted in FIG. 4.

Referring now to FIGS. 1 and 2, there is shown a prior art X-ray system 1 employing an X-ray image intensifier tube 2. Such a system is described in an article entitled, "X-ray Image Intensification With a Large Diameter Image Intensifier Tube," appearing in the American Journal of Roentgenology Radium Therapy and Nuclear Medicine, volume 85, pages 323-341 of February 1961. Briefly, an X-ray generator 3 serves to produce and direct a beam of X-rays onto an object 4 to be X-rayed. The image intensifier tube 2 is disposed to receive the X-ray image of the object 4.

The image intensifier tube 2 includes a dielectric vacuum envelope 5 as of glass approximately 17 inches long and 10 inches in diameter. The pick-up face portion 6 of the tube 2 comprises a spherical X-ray transparent portion of the envelope 5, as of aluminum or conductive glass, which is operated at cathode potential. An image pick-up screen 7 of X-ray sensitive particulated phosphor such as ZnS is coated onto the inside spherical surface of the envelope portion 5 to a thickness as of 0.020".

A chemically inert optically transparent buffer layer 8 is coated over the phosphor layer 7. A photo-cathode layer 9 is formed over the buffer layer 8.

In operation, the X-rays penetrate the object 4 to be observed. The local X-ray attenuation depends on both the thickness and atomic number of the elements forming the object under observation. Thus, the intensity pattern in the X-ray beam after penetration of the object 4 contains information concerning the structure of the object. The X-ray image passes through the X-ray transparent envelope section 5 and falls upon the X-ray sensitive phosphor layer 7 wherein the X-ray photons are absorbed and re-emitted as optical photons, typically in the blue frequency range. The optical photons pass through the transparent buffer 8 to the photo-cathode 9 wherein they produce electrons. The electrons are emitted from the photo-cathode in a pattern or image corresponding to the original X-ray image. The electrons are accelerated to a high velocity, as of 30 kv, within the tube 2 and are focused through an anode structure 12 onto a fluorescent screen 13 for viewing by the eye or other suitable optical pick-up device. Electron focusing electrodes 14 are deposited on the interior surfaces of the tube 2 to focus the electrons through the anode 12.

In the intensifier tube, one 50 kev. photon of X-ray energy absorbed by the X-ray sensitive pick-up screen produces about 2000 photons of blue light. These 2000 photons of blue light produce about 400 electrons when absorbed in the photo-emitter layer 9. The 400 electrons emitted from the photo-cathode produce about 400,000 photons of light in the visible band when absorbed by the fluorescent viewing screen 13. Thus, the X-ray image is converted to the visible range and greatly intensified for viewing.

One of the problems with the prior art intensifier tube 2 is that the particulated pick-up screen has less than optimum resolution due to the fact that the particulated material has about one-half the density of the material in bulk form. Thus, to provide a certain probability of stopping or absorbing an X-ray photon, the particulated layer 7 must have about twice the thickness of such a layer if it had bulk density. The thicker the layer 7 the poorer its X-ray resolution. Moreover, the particulated material serves to scatter the emitted optical photons, thereby still further reducing resolution.

In addition, it is desirable to utilize a pick-up screen material having a greater intrinsic stopping or absorbing power for X-rays. Such improved materials include the alkali metal halides such as, for example, CsI, KI, NaI, RbI, CsBr, and LiI. These improved materials such as CsI and NaI are obtainable in bulk slab form from Harshaw Chemical Company of Cleveland, Ohio. However, when they are distorted from the slab form into the spherical slab form, to conform to the spherical pick-up face 6 of the image intensifier tube 2, it is expected that the conversion efficiency and, hence, resolution of the converted X-ray image is deleteriously affected.

Referring now to FIGS. 3-5 there is shown a section of the X-ray pick-up screen formed in accordance with the methods of the present invention. More particularly, the alkali metal halide pick-up screen layer 16 is formed on the spherical X-ray transparent substrate member 5 by evaporation in vacuum.

In a first method, the substrate member 5 is cleaned and disposed in a vacuum chamber 17 of a vacuum evaporator 18. A crucible 19 containing the activated alkali metal halide phosphor 21 in bulk form is heated to a temperature sufficient to evaporate the phosphor material as by an electrical heating element 22. The evaporated activated alkali halide is condensed (deposited) on the substrate 5 to the desired thickness as of 0.010" for an X-ray image intensifier and to 0.060" for a gamma ray intensifier. As used herein, "X-ray" is defined to include X-rays and other high energy radiation including gamma ray radiation.

The bulk activated alkali halide may include any one of a number of different activators to render the pick-up screen 16 fluorescent upon absorption of X-rays at room

temperature. For example, CsI may include TiI or NaI, Na or LiI as activators.

After the screen layer 16 has been deposited it is preferably annealed to remove any residual minute plastic deformations thereof because such deformations have an adverse effect upon quantum conversion efficiency. A suitable annealing process is to heat the screen 16 as by heater 23 in vacuum to within 10° C. of the melting point of the screen material for 0.5 to 2.0 hours and then cool the screen 16 through to 400° C. in 10 hours and then cool to room temperature in another 10 hours.

An ultra clean vacuum pump 24 is connected into the evaporation chamber 17 to maintain the vacuum within the system at about 10<sup>-9</sup> torr during the evaporation process.

The deposited layer of phosphor 16 is polycrystalline and has a density approximately equal to the bulk density of the alkali metal halide material. The polycrystalline nature of the vacuum evaporated alkali metal halide material is well known. See, for example, The Physical Review, volume 51, No. 5, of Mar. 1, 1937, pages 293-298, especially pages 295-297. Therefore, the X-ray stopping or absorption power of the layer 16 is substantially improved for a given thickness as compared to the prior particulated phosphor screens. Thus, the thickness of the layer 16 can be reduced compared to the prior screens, thereby providing improved resolution. Moreover, the spherical shape of the layer 16 does not interfere with resolution as would be expected to be encountered if a slab of the alkali halide material were shaped to conform to the spherical substrate 6.

A second method for forming the evaporated pick-up screen 16 is essentially the same as the first method except that the activator material is not incorporated in the bulk phosphor material 21 to be evaporated. Instead, the activator material 26 is simultaneously evaporated from a second crucible 27 which is heated by a separate heater 28. This method provides better control over relative rates of deposition of the alkali halide and its activator in order to assure a better control over the distribution of the activator in the deposited screen layer 16. As an alternative to employing the second crucible 27, the activator is vaporized in the chamber 17 to form a vapor in equilibrium. The alkali halide material, without the activator, is then evaporated through the activator vapor and, thus, co-deposited with the activator vapor on the substrate 6. A third method for forming the screen layer 16 is essentially the same as the second method except that the activator is post evaporated to form a layer upon the previously deposited layer of alkali metal halide screen material. The activator is then diffused into the alkali metal halide screen layer by annealing as previously described with regard to the first method.

A fourth method for forming the pick-up screen layer 16 is essentially the same as any one of the aforescribed methods except that the materials to be evaporated from a heated crucible are instead flash evaporated. More particularly, an evaporation plate 31 is heated by a heater 32 to a temperature well in excess of the evaporation temperature of the constituents of the material to be evaporated. Pellets 33 of the material to be evaporated which in some methods, as aforescribed, include the alkali metal halide with the activator incorporated therein, and in others of the aforescribed methods have the activator separately evaporated, are dropped upon the plate 31 for flash evaporation. The evaporated material is collected on the substrate 5 to form the pick-up screen layer 16. For the methods wherein the activator is separately evaporated the proportions of activator and alkali metal halide, in the resultant deposited layer 16, are controlled by controlling the rate at which the separate activator and alkali metal halide pellets are dropped upon the evaporation plate 31. The resultant screen layer 16 may be heat treated or annealed, as aforescribed,

to obtain a more uniform distribution of the activator within the alkali metal halide material and to remove residual plastic deformation.

Still other methods for evaporation of the alkali metal halide material in vacuum onto the curved face plate 6 include electron beam and laser beam evaporation methods.

The buffer layer 8 is formed over the pick-up screen layer 16 by evaporating a chemically inert and optically transparent material over the layer 16 to a thickness less than 10,000 Å. and preferably 1000 Å. or less. Suitable buffer materials include magnesium oxide, aluminum oxide and lithium fluoride. Such materials are evaporated in vacuum in the same manner as previously described for evaporation of the pick-up screen materials. As an alternative, the buffer layer 8 is formed, in some instances, by evaporating the metal constituent such as aluminum or magnesium and then reacting the deposited metal film with the other constituent of the buffer such as oxygen gas, which is introduced into the vacuum chamber 17, to form the buffer layer 8.

The photo-cathode layer 9, as of  $\text{Cs}_3\text{Sb}$ , is deposited over the buffer layer 8 by conventional vacuum evaporation methods for forming such cathodes. Such a method is described in a book entitled, "Photoelectronic Materials and Devices" published by D. Van Nostrand Company, Inc. in 1965 at pp. 200-201.

One advantage of the aforescribed vacuum evaporation methods for forming the pick-up screen 16 and subsequent buffer and photo-cathode layers 8 and 9, respectively, is that such methods are all performed in vacuum such that they lend themselves to a production machine which performs the successive steps in vacuum without having to take the parts into air for performing successive steps in the manufacture.

Since many changes could be made in the above construction and many apparently widely different embodiments of this invention can be made without departing from the scope thereof it is intended that all matter contained in the above description or shown in the accompanying drawings shall be interpreted as illustrative and not in a limiting sense.

What is claimed is:

1. In a method for making an X-ray pick-up screen of improved resolution and quantum conversion efficiency for an evacuated X-ray image intensifier tube the steps of, vaporizing in vacuum an alkali metal halide material selected from the group consisting of CsI, NaI, LiI, KI, CsBr and RbI, condensing in vacuum the vaporized material on a substrate to form on said substrate a layer having a density approximately equal to that of the bulk alkali metal halide material, and incorporating an activator material into the condensed layer forming an activated X-ray sensitive scintillator for the X-ray image tube.

2. The method of claim 1 wherein the step of incorporating said activator material into said condensed layer includes the steps of, co-evaporating and co-condensing said activator material and said alkali metal halide material in vacuum onto said substrate.

3. The method of claim 1 wherein the step of incorporating, said activator material into said condensed layer includes the step of, evaporating in vacuum said alkali metal halide material having said activator material incorporated therein as an activator for said alkali metal halide such that the material to be evaporated is pre-activated with said activator material.

4. The method of claim 1 wherein said alkali metal halide material is CsI.

5. The method of claim 4 wherein said photocathode 70 includes cesium and antimony.

6. The method of claim 1 wherein said alkali metal halide is CsI and said activator material is selected from the group consisting of Na and NaI.

7. The method of claim 1 wherein the step of incorporating said activator material into said condensed layer includes the step of, coating the surface of said condensed layer with said activator material and heating said coated layer to diffuse said activator material into said layer.

8. The method of claim 7 wherein the step of coating the surface of said condensed layer with said activator material includes the step of, evaporating in vacuum said activator material, and condensing said evaporated activator material on said condensed layer of said alkali metal halide material.

9. The method of claim 1 including the step of, annealing said condensed layer of alkali metal halide material.

10. The method of claim 1 wherein said activator material is selected from the group consisting of TlI, NaI, Na, and LiI.

11. The method of claim 1 wherein the substrate is dish-shaped to form a dish-shaped scintillator layer.

12. The method of claim 1 including the step of, depositing a photocathode material overlaying said scintillator which is sensitive to the X-ray induced scintillations of said scintillator for converting the scintillated image into an electron image to be emitted into the evacuated X-ray image intensifier tube.

13. The method of claim 1 wherein said X-ray pick-up screen includes a polycrystalline X-ray sensitive scintillator, and wherein the step of condensing the vaporized material includes, condensing the vaporized material in vacuum on the substrate forming on said substrate a polycrystalline layer, and wherein the step of incorporating said activator into said condensed layer includes, incorporating said activator into said polycrystalline layer for activating same forming the activated X-ray sensitive polycrystalline scintillator.

14. The method of claim 1 wherein said activated X-ray sensitive scintillator layer is of a thickness greater than 0.0005 inch.

15. In a method for making an evacuated X-ray image intensifier tube, the steps of; vaporizing in vacuum an alkali metal halide material selected from the group consisting of CsI, NaI, LiI, KI, CsBr, and RbI; condensing in vacuum the vaporized material on a substrate to form a polycrystalline layer on said substrate, said layer having a density approximately equal to that of the bulk alkali metal halide material; incorporating an activator material into the condensed layer forming an activated X-ray sensitive polycrystalline scintillator; and disposing said activated X-ray sensitive polycrystalline scintillator screen within an evacuable envelope of an X-ray intensifier tube for receiving an X-ray image to be intensified.

References Cited

UNITED STATES PATENTS

|           |        |                      |            |
|-----------|--------|----------------------|------------|
| 3,023,313 | 2/1962 | De La Mater et al.   | 117-33.5 X |
| 2,936,246 | 5/1960 | Coghill -----        | 117-33.5 X |
| 2,673,816 | 3/1954 | Neuhaus et al. ___   | 117-33.5 X |
| 2,789,062 | 4/1957 | Cusano et al. ___    | 117-33.5 X |
| 2,798,823 | 7/1957 | Harper -----         | 117-33.5   |
| 2,676,113 | 4/1954 | Jervis -----         | 117-33.5 C |
| 2,898,225 | 8/1959 | Rychlewski et al. __ | 117-33.5 C |
| 2,903,378 | 9/1959 | Rychlewski -----     | 117-33.5 C |

RALPH S. KENDALL, Primary Examiner

U.S. CL. X.R.

117-106 R; 250-80, 213

UNITED STATES PATENT OFFICE  
CERTIFICATE OF CORRECTION

Patent No. 3,795,531 Dated March 5, 1974

Inventor(s) William E. Spicer

It is certified that error appears in the above-identified patent and that said Letters Patent are hereby corrected as shown below:

Column 1, line 33, After "application." insert --This application claims a method of fabrication the device of the invention is claimed in division hereof, Serial No. 281,905, filed 18 August 1972.--

Claim 1, line 10, Change "forming" to --to form--.

Claim 11, line 2, After "dish-shaped" insert --so as--.

Claim 12, line 3, Change "which is" to --, said material being--.

Claim 13, line 5, After "substrate", 1st occ. insert -- , --  
line 9, Change "forming the" to --so as to form an--.

Claim 15, line 9, Change "forming" to --to form--.

Claim 3, lines 1-2, After "incorporating" delete ",",.

Signed and sealed this 29th day of October 1974.

SEAL)  
ttest:

COY M. GIBSON JR.  
ttesting Officer

C. MARSHALL DANN  
Commissioner of Patents